# EUROPEAN PATENT SPECIFICATION

(11) **EP 3 812 477 B1**
(45) Date of publication and mention of the grant of the patent: **11.01.2023**
(21) Application number: 19306367.4
(22) Date of filing: 21.10.2019
(51) Int. Cl.: C22C 5/02, A44C 27/00, C22F 1/14

(54) **METAL ALLOY COMPRISING GOLD**
GOLDHALTIGE METALLLEGIERUNG
ALLIAGE MÉTALLIQUE COMPRENANT DE L'OR

(43) Date of publication of application: 28.04.2021
(73) Proprietor: Richemont International SA, 1752 Villars-sur-Glane (CH)
(72) Inventor: LALIRE, Fanny, 90000 BELFORT (FR); THEDY, Louis, 69100 VILLEURBANNE (FR)
(74) Representative: Ipsilon

(56) References cited:
- EP-A1- 0 008 975
- EP-A1- 1 010 768
- EP-A1- 1 512 765
- WO-A1-2019/175826
- CN-A- 108 588 467
- CN-A- 108 588 467
- GB-A- 372 236
- JP-A- 2001 207 226
- US-A- 5 221 207
- US-A1- 2014 328 718
- US-A1- 2018 171 436
- DAVID J KINNEBERG ET AL: "Origin and effects of impurities in high purity gold", GOLD BULLETIN, WORLD GOLD COUNCIL, LONDON, GB , vol. 31, no. 2 1 July 1998 (1998-07-01), pages 58-67, XP002545057, ISSN: 1027-8591 Retrieved from the Internet: URL:http://www.goldbulletin.org/assets/fil e/goldbulletin/downloads/Kinneber_2_31.pdf [retrieved on 1998-07-01]

## Description

The present invention relates to a metal alloy comprising several metallic elements including gold (Au), and a process of manufacturing said metal alloy.

More particularly, the metal alloy is used to manufacture luxury goods.

It exists several types of metal alloys used to manufacture luxury goods such as a time-piece or a jewel. One can cite the document WO 2019/073023 concerning a metal alloy comprising at least four metallic elements such as scandium (Sc), aluminum (Al), titanium (Ti) and lithium (Li). The published international application WO 2019/175826 A1 concerns a gold alloy containing additions of Cu, Ag, Pd and Fe which provides a high level of discoloration resistance for use in jewelry applications.

However, despite the various metal alloys which are commercially available, there is still a need to have new alternative metal alloys able to be used in the domain of luxury goods, with optimized properties.

In this respect, the present invention seeks to provide a new metal alloy, having optimized mechanical properties, while being easy to shape.

To this end, an object of the present invention is a metal alloy according to claim 1.

The present invention advantageously provides a metal alloy with an improved hardness, while guaranteeing a good ductility. More particularly, the hardness of the metal alloy can advantageously be of at least 150 Vickers hardness (HV) (i.e. kilograms-force per square millimeter), more preferably of at least 200 HV, and even more preferably of at least 250 HV.

The metal alloy is also advantageously easy to shape, especially to manufacture luxury good.

The metal alloy of the present invention has advantageously a high entropy.

More particularly, the entropy of the metal alloy can be of at least 0.69R, more preferably at least 1.00R, and even more preferably at least 1.20R, R being the molar gas constant.

The entropy can be easily determined by the man skilled in the art, according to the well-known Boltzmann's definition related to the following equation: ΔS_{conf} = - RΣXᵢIn(Xᵢ), where Xᵢ represents the atomic fraction of element i and R is the molar gas constant.

A high entropy can favor the formation of a solid solution, which may help to improve the ductility of the metal alloy.

The metal alloy of the present invention can be a solid solution. A solid solution is well known in the art and can be considered as a solid-state solution comprising several metallic elements wherein the metallic elements remain in a single homogeneous phase in the metal alloy. Thus, the metal alloy of the invention can preferably be a single-phase alloy.

In the present invention, gold (Au) is used as main metallic element among the at least five metallic elements constituting the metal alloy.

Indeed, among the at least five metallic elements, the metal alloy comprises an amount of gold (Au) superior or equal to 58.3 % by weight over the total weight of the metal alloy.

An amount of gold (Au) of at least 58.3 % by weight over the total weight of the metal alloy is particularly advantageous since it corresponds to an amount of 583 ‰ (per mille) by weight of gold (Au) over the total weight of the metal alloy. With this lower limit of at least 583 ‰ by weight of gold (Au), the metal alloy can be considered as a precious material of 14-karat gold (i.e. 14k), under the karat standard system for gold alloy.

In a particular embodiment, the metal alloy can comprise at least 70.0 % by weight of gold (Au), and more preferably 75.0 % by weight of gold (Au), over the total weight of the metal alloy.

An amount of gold (Au) of at least 75.0 % by weight over the total weight of the metal alloy is particularly advantageous since it corresponds to an amount of 750 ‰ (per mille) by weight of gold (Au) over the total weight of the metal alloy. With this lower limit of at least 750 ‰ by weight of gold (Au), the metal alloy can be considered as a precious material of 18-karat gold (i.e. 18k), under the karat standard system for gold alloy.

In the present invention, the metal alloy comprises at least four metallic elements different from gold (Au), each of said four metallic elements being in an amount from 5.0 to 30.0 atomic percent (at.%).

The atomic percent of each metallic elements constituting the metal alloy is expressed over the total atomic percent (100%) of the metallic elements constituting the metal alloy.

The four metallic elements are selected among silver (Ag), aluminum (Al), manganese (Mn), copper (Cu), palladium (Pd), iron (Fe), and chromium (Cr), platinum (Pt), and cobalt (Co).

In a first embodiment, the four metallic elements can be copper (Cu), silver (Ag), manganese (Mn), and aluminum (Al).

According to this first embodiment, the metal alloy can be for example, in at%, Au_{34.4}Cu_{25.9}Ag_{22.8}Mn_{9.6}Al_{7.3} or Au_{52.5}Cu_{20.3}Ag_{15.2}Mn_{6.5}Al_{5.5}.

In a second embodiment, the four metallic elements can be palladium (Pd), silver (Ag), chromium (Cr), and iron (Fe).

According to this second embodiment, the metal alloy can be for example, in at%, Au_{36.6}Pd_{16.4}Ag_{16.2}Cr_{15.4}Fe_{15.4}.

In a third embodiment, the four metallic elements can be silver (Ag), chromium (Cr), palladium (Pd), and cobalt (Co).

According to this third embodiment, the metal alloy can be for example, in at%, Au_{38.0}Ag_{15.5}Cr_{15.5}Pd_{15.5}Co_{15.5}.

In a fourth embodiment, the four metallic elements can be silver (Ag), cobalt (Co), palladium (Pd), and iron (Fe).

According to this fourth embodiment, the metal alloy can be for example, in at%, Au_{38.0}Ag_{15.5}Co_{15.5}Pd_{15.5}Fe_{15.5}.

In a fifth embodiment, the four metallic elements can be silver (Ag), platinum (Pt), palladium (Pd), and iron (Fe).

According to this fifth embodiment, the metal alloy can be for example, in at%, Au_{67.0}Ag_{8.25}Pt_{8.25}Pd_{8.25}Fe_{8.25}.

The gold (Au) used in the metal alloy of the invention can preferably have a purity of at least 99.5 %, and more preferably of at least 99.9 % and even more preferably of at least 99.99 %.

The metallic elements different from gold (Au) can also have a purity of at least 99.0 %, and more preferably of at least 99.9 %.

Another object of the present invention is a process of manufacturing said metal alloy, the process comprising the following steps:
i. forming a molten alloy comprising gold (Au) and the at least four metallic elements different from gold,
ii. cold rolling the alloy obtained in step i, and
iii. optionally, annealing the alloy obtained in step ii.

The step i can include a mixture of the metallic elements as such and/or one or several pre-alloy(s).

The step i can be done in using an arc furnace, classically in placing the metallic elements and/or the pre-alloy(s) in a crucible, and submitting then with an electric arc producing a temperature of up to 3000°C. This process makes it possible to produce alloys from pure elements with different melting temperatures. The metallic element mixture can then be cooled to room temperature (around 25°C).

In another embodiment, the step i can be done in using an induction furnace, classically in placing the metallic elements and/or the pre-alloy(s) in a crucible, and submitting then with an induction heating. The metallic element mixture can then be cooled to room temperature (around 25°C).

A pre-alloy can be a mixture of at least two metallic elements having similar melting temperature. For example, a pre-alloy can be formed with two metallic elements having a melting temperature difference inferior or equal to 150°C, and more preferable inferior or equal to 100°C.

The pre-alloys can be formed in using an arc furnace. The metallic element mixture can then be cooled to room temperature (around 25°C).

The alloy obtained in step i is then rolled in order to increase its mechanical properties and modify its internal structure. The rolling step can be done at room temperature (around 25°C) in using a rolling mill. The rolling step can usually be performed after cooling to room temperature (around 25°C) the alloy obtained in step i.

The step iii can be advantageously done to improve the yield strength and the hardness of the alloy, especially when several cold rolling passes are done.

The temperature and annealing time depend on the nature of the alloy, the rate of cold work previously applied and the properties required, according to the conditions well-known in the art.

For example, the annealing step can be done at a temperature around 750°C, during 30 minutes.

In a particular embodiment, when the step iii is performed, the step iii can be followed by one or several steps of cold rolling as detailed in step ii.

Another object of the present invention is an item obtained from the metal alloy.

The item can comprise or consist of the metal alloy according to the present invention. Accordingly, the metal alloy can be used in order to manufacture luxury goods, such as for example a time-piece and/or a jewel. The time-piece and/or the jewel can have a part or a component comprising the metal alloy according to the present invention.

More particularly, the item according to the present invention can be a jewel, a leather good, or a clothing accessory. It may also be a watch, a writing accessory, or a decorative item.

For instance, the item can be any of the followings: ring; ear ring; necklace; bracelet; pendant; watch such as case, bezel, caseback, crown, bracelet links, clasp, buckle, automatic movement rotor; buckle (e.g. belt or purse); tie bar; cuff links; money clip; hair pin; pen; paper knife.

The present invention will become more fully understood from the examples given herein below, which are given by way of illustration only, and thus, which are not limits of the present invention.

### Examples:

### 1. Preparation of the metal alloys according to the invention

Different metal alloys according to the present invention, i.e. Metal alloy 1, Metal alloy 2, Metal alloy 3, Metal alloy 4 and Metal alloy 5, have been prepared and are respectfully gathered in the following Tables 1 to 5.

The amounts in Tables 1 to 5 are expressed:
- in atomic percent (at%) over all the metallic element constituting the metal alloy, and
- in weight percent (wt%) over the total weight of the metal alloy.

According to the amount of gold, Metal alloy 1, Metal alloy 3 and Metal alloy 4 can be considered as a precious alloy of 14-karat gold, and Metal alloy 2 and Metal alloy 5 can be considered as a precious alloy of 18-karat gold.

**Table 1**

| Metal alloy 1 | Au | Cu | Ag | Mn | Al | Total |
|---|---|---|---|---|---|---|
| Atomic percent (at%) | 34.4 | 25.9 | 22.8 | 9.6 | 7.3 | 100 |
| Weight percent (wt%) | 58.4 | 14.2 | 21.2 | 4.5 | 1.7 | 100 |

**Table 2**

| Metal alloy 2 | Au | Cu | Ag | Mn | Al | Total |
|---|---|---|---|---|---|---|
| Atomic percent (at%) | 52.5 | 20.3 | 15.2 | 6.5 | 5.5 | 100 |
| Weight percent (wt%) | 75.1 | 9.3 | 12.0 | 2.6 | 1.0 | 100 |

**Table 3**

| Metal alloy 3 | Au | Pd | Ag | Cr | Fe | Total |
|---|---|---|---|---|---|---|
| Atomic percent (at%) | 36.6 | 16.4 | 16.2 | 15.4 | 15.4 | 100 |
| Weight percent (wt%) | 58.3 | 14.1 | 14.1 | 6.5 | 7.0 | 100 |

**Table 4**

| Metal alloy 4 | Au | Ag | Cr | Pd | Co | Total |
|---|---|---|---|---|---|---|
| Atomic percent (at%) | 38.0 | 15.5 | 15.5 | 15.5 | 15.5 | 100 |
| Weight percent (wt%) | 59.8 | 13.3 | 6.4 | 13.2 | 7.3 | 100 |

**Table 5**

| Metal alloy 5 | Au | Ag | Pt | Pd | Fe | Total |
|---|---|---|---|---|---|---|
| Atomic percent (at%) | 67.0 | 8.25 | 8.25 | 8.25 | 8.25 | 100 |
| Weight percent (wt%) | 77.47 | 5.22 | 9.45 | 5.15 | 2.71 | 100 |

The preparation of the metal alloys gathered in Tables 1-5 is described as follows.

Firstly, a molten alloy is formed (step i) in using an arc furnace, in placing and mixing all the metallic elements constituting a metal alloy, in a crucible.

After cooling to room temperature (around 25°C) the alloy obtained in step i, a rolling step is performed (step ii) at room temperature (around 25°C), with several passes, in using a roller mill.

The rolling step is of:
- 83% to obtain the Metal alloy 1,
- 90% to obtain the Metal alloy 2,
- 70% to obtain the Metal alloy 3,
- 70% to obtain the Metal alloy 4,
- 60% to obtain the Metal alloy 5,

The rolled alloy is under the form of a bar.

### 2. Characterization of the metal alloys

Some properties of the metal alloys obtained in the preparation as described above can be easily determined, such as entropy, ΔE and hardness.

### 2.1. Determination of the entropy

The entropy is determined following the equation ΔS_{conf} = - RΣXᵢIn(Xᵢ), where Xᵢ represents the atomic fraction of element i and R is the molar gas constant.

### 2.2. Determination method of the color

In order to evaluate the color of a metal alloy, the CIELAB coordinates, which are well known as color space specified by the International Commission on Illumination (known in French with the acronym CIE), are used.

The three coordinates of CIELAB represent the lightness of the color (L^{∗} = 0 yields black and L^{∗} = 100 indicates diffuse white), its position between red/magenta and green (a^{∗}, negative values indicate green while positive values indicate magenta) and its position between yellow and blue (b^{∗}, negative values indicate blue and positive values indicate yellow).

To compare two different colors, or to characterize the evolution of a sample, the expression "ΔE^{∗}" can be used. ΔE^{∗} corresponds to the distance between two colors placed in the CIELAB color space which is calculated with the formula of the Euclidian distance. ΔE^{∗} can also be written ΔE or ΔE_{ab}.

ΔE^{∗} is classically known as follows: ${ΔE}^{*} = \sqrt{{\left({L}_{2}^{*}-{L}_{1}^{*}\right)}^{2} + {\left({a}_{2}^{*}-{a}_{1}^{*}\right)}^{2} + {\left({b}_{2}^{*}-{b}_{1}^{*}\right)}^{2}}$ wherein: ${L}_{1}^{∗} , {a}_{1}^{∗} , {b}_{1}^{∗}$ are the coordinates of the first color to compare, and ${L}_{2}^{∗}$, ${a}_{2}^{∗} , {b}_{2}^{∗}$ are the coordinates of the second color to compare.

The illuminant used to evaluate the metal alloy color is the CIE D65 standard illuminant, with a viewing angle of 10°.

The evolution of the metal alloy color is studied according to the test Tuccillo-Nielsen wheel method, which aims at evaluating the tarnish testing of an alloy in contact with the skin. In this respect, the metal alloy is immersed during 30 seconds in artificial sweet and then dried in the open air during 30 seconds, in a continuous way. The artificial sweet composition used for the test is the composition according to European Committee for Standardization EN 1811, which is a solution of 0.5% NaCl, 0.1% urea and 0.1% lactic acid, with a pH adjusted to 6.5 using NH₄OH. Color measurements are taken at t=0, 4, 7, 15 and 25 days.

Finally, ΔE between t=0 and t=25 days is calculated. Hence, a low ΔE means a low color evolution.

### 2.3. Determination method of the hardness

In order to evaluate the hardness of a metal alloy, a Vickers microhardness tester on polished samples has been used. The samples have been indented linearly on the surfaces at five different positions and the average have been recorded. The indentation load was 2 kg with an indentation time of 10 seconds.

In the present invention, the hardness of the metal alloy can advantageously be of at least 200 HV, more preferably of at least 250 HV, and even more preferably of at least 300 HV. Said hardness (i.e. final hardness) is more particularly the one determined on the metal alloy obtained after the steps i, ii and optionally iii.

Another advantage is that the alloy obtained before the step ii can have a hardness of at least 200 HV. Said hardness (i.e. raw hardness) is more particularly the one determined on the alloy obtained in step i, or in other words, before step ii.

### 2.4. Results

In order to show the effects of the present invention, a comparative example has been performed (Metal alloy 6), and is gathered in the below table 6.

The amounts in Table 6 are expressed in weight percent (wt%) over the total weight of the metal alloy.

**Table 6**

| Metal alloy 6 | Au | Ag | Cu | Total |
|---|---|---|---|---|
| Weight percent (wt%) | 58.5 | 26.5 | 15.0 | 100 |

The preparation of said Metal alloy 6 is similar to the preparation described in the above item 1, except that the rolling step (step ii) is of 75%.

The results are gathered in the following Table 7.

**Table 7**

| | Metal alloy 1 | Metal alloy 2 | Metal alloy 3 | Metal alloy 4 | Metal alloy 5 | Metal alloy 6 |
|---|---|---|---|---|---|---|
| Entropy | 1.47R | 1.29R | 1.47R | 1.52R | 1.29R | 0.99R |
| ΔE | 2.57 | 3.66 | Not measured | Not measured | 1.02 | 3.53 |
| Raw hardness | 230 | 150 | 194 | 188 | 228 | 175 |
| Final hardness | 330 | 320 | 253 | 237 | 246 | 260 |

## Claims

1. Metal alloy comprising at least four metallic elements different from gold (Au), **characterized in that** the metal alloy consists of gold (Au) in an amount of at least 58.3 % by weight over the total weight of the metal alloy and of 5.0 to 30.0 atomic percent of each of said four metallic elements, the four metallic elements being selected among silver (Ag), aluminum (Al), manganese (Mn), copper (Cu), palladium (Pd), iron (Fe), chromium (Cr), platinum (Pt), and cobalt (Co).

2. Metal alloy according to claim 1, **characterized in that** the metal alloy comprises at least 75.0 % by weight of gold (Au), over the total weight of the metal alloy.

3. Metal alloy according to claim 1 or 2, **characterized in that** the four metallic elements are copper (Cu), silver (Ag), manganese (Mn), and aluminum (Al).

4. Metal alloy according to claim 1 or 2, **characterized in that** the four metallic elements are palladium (Pd), silver (Ag), chromium (Cr), and iron (Fe).

5. Metal alloy according to claim 1 or 2, **characterized in that** the four metallic elements are silver (Ag), chromium (Cr), palladium (Pd), and cobalt (Co).

6. Metal alloy according to claim 1 or 2, **characterized in that** the four metallic elements are silver (Ag), cobalt (Co), palladium (Pd), and iron (Fe).

7. Metal alloy according to claim 1 or 2, **characterized in that** the four metallic elements are silver (Ag), platinum (Pt), palladium (Pd), and iron (Fe).

8. Process of manufacturing a metal alloy according to any one of the preceding claims, **characterized in that** the process comprises the following steps:
i. forming a molten alloy comprising gold (Au) and the at least four metallic elements different from gold,
ii. cold rolling the alloy obtained in step i, and
iii. optionally, annealing the alloy obtained in step ii.

9. Time-piece or jewel having a part or a component comprising the metal alloy according to any one of claims 1 to 8.

## Patentansprüche

1. Metalllegierung, die zumindest vier metallische Elemente umfasst, bei denen es sich nicht um Gold (Au) handelt, **dadurch gekennzeichnet, dass** die Metalllegierung aus Gold (Au) in einer Menge von zumindest 58,3 Gew.-% in Bezug auf das Gesamtgewicht der Metalllegierung und aus 5,0 bis 30,0 Atomprozent jedes der vier metallischen Elemente besteht, wobei die vier metallischen Elemente aus Silber (Ag), Aluminium (AI), Mangan (Mn), Kupfer (Cu), Palladium (Pd), Eisen (Fe), Chrom (Cr), Platin (Pt) und Kobalt (Co) ausgewählt sind.

2. Metalllegierung nach Anspruch 1, **dadurch gekennzeichnet, dass** die Metalllegierung zumindest 75,0 Gew.-% Gold (Au) in Bezug auf das Gesamtgewicht der Metalllegierung umfasst.

3. Metalllegierung nach Anspruch 1 oder 2, **dadurch gekennzeichnet, dass** die vier metallischen Elemente Kupfer (Cu), Silber (Ag), Mangan (Mn) und Aluminium (AI) sind.

4. Metalllegierung nach Anspruch 1 oder 2, **dadurch gekennzeichnet, dass** die vier metallischen Elemente Palladium (Pd), Silber (Ag), Chrom (Cr) und Eisen (Fe) sind.

5. Metalllegierung nach Anspruch 1 oder 2, **dadurch gekennzeichnet, dass** die vier metallischen Elemente Silber (Ag), Chrom (Cr), Palladium (Pd) und Kobalt (Co) sind.

6. Metalllegierung nach Anspruch 1 oder 2, **dadurch gekennzeichnet, dass** die vier metallischen Elemente Silber (Ag), Kobalt (Co), Palladium (Pd) und Eisen (Fe) sind.

7. Metalllegierung nach Anspruch 1 oder 2, **dadurch gekennzeichnet, dass** die vier metallischen Elemente Silber (Ag), Platin (Pt), Palladium (Pd) und Eisen (Fe) sind.

8. Verfahren zum Herstellen einer Metalllegierung nach einem der vorstehenden Ansprüche, **dadurch gekennzeichnet, dass** das Verfahren die folgenden Schritte umfasst:
i. Bilden einer geschmolzenen Legierung, die Gold (Au) und die zumindest vier metallischen Elemente, bei denen es sich nicht um Gold handelt, umfasst,
ii. Kaltwalzen der in Schritt i. erhaltenen Legierung, und
iii. wahlweise Glühen der in Schritt ii. erhaltenen Legierung.

9. Uhr oder Schmuckstück mit einem Teil oder einer Komponente, der bzw. die die Metalllegierung nach einem der Ansprüche 1 bis 8 umfasst.

## Revendications

1. Alliage métallique comprenant au moins quatre éléments métalliques différents de l'or (Au), **caractérisé en ce que** l'alliage métallique est constitué d'or (Au) en une quantité d'au moins 58,3 % en poids par rapport au poids total de l'alliage métallique et de 5,0 à 30,0 pour cent atomiques de chacun desdits quatre éléments métalliques, les quatre éléments métalliques étant choisis parmi l'argent (Ag), l'aluminium (Al), le manganèse (Mn), le cuivre (Cu), le palladium (Pd), le fer (Fe), le chrome (Cr), le platine (Pt) et le cobalt (Co).

2. Alliage métallique selon la revendication 1, **caractérisé en ce que** l'alliage métallique comprend au moins 75,0 % en poids d'or (Au), par rapport au poids total de l'alliage métallique.

3. Alliage métallique selon la revendication 1 ou 2, **caractérisé en ce que** les quatre éléments métalliques sont le cuivre (Cu), l'argent (Ag), le manganèse (Mn) et l'aluminium (Al).

4. Alliage métallique selon la revendication 1 ou 2, **caractérisé en ce que** les quatre éléments métalliques sont le palladium (Pd), l'argent (Ag), le chrome (Cr) et le fer (Fe).

5. Alliage métallique selon la revendication 1 ou 2, **caractérisé en ce que** les quatre éléments métalliques sont l'argent (Ag), le chrome (Cr), le palladium (Pd) et le cobalt (Co).

6. Alliage métallique selon la revendication 1 ou 2, **caractérisé en ce que** les quatre éléments métalliques sont l'argent (Ag), le cobalt (Co), le palladium (Pd) et le fer (Fe).

7. Alliage métallique selon la revendication 1 ou 2, **caractérisé en ce que** les quatre éléments métalliques sont l'argent (Ag), le platine (Pt), le palladium (Pd) et le fer (Fe).

8. Procédé de fabrication d'un alliage métallique selon l'une quelconque des revendications précédentes, **caractérisé en ce que** le procédé comprend les étapes suivantes :
i. formation d'un alliage fondu comprenant de l'or (Au) et les au moins quatre éléments métalliques différents de l'or,
ii. laminage à froid l'alliage obtenu à l'étape i, et
iii. facultativement, recuit de l'alliage obtenu à l'étape ii.

9. Appareil horaire ou bijou comportant une pièce ou un composant comprenant l'alliage métallique selon l'une quelconque des revendications 1 à 8.
